

A. G. BETTS.

## ELECTROLYTICALLY REFINING SILVER.

APPLICATION FILED MAR. 8, 1905.



Witnesses

Edward J. Kenne  
Frederick Clark

Inventor

Aaron Gardner Betts

# UNITED STATES PATENT OFFICE.

ANSON GARDNER BETTS, OF TROY, NEW YORK.

## ELECTROLYTICALLY REFINING SILVER.

No. 795,887.

Specification of Letters Patent.

Patented Aug. 1, 1905.

Application filed March 8, 1905. Serial No. 249,054.

*To all whom it may concern:*

Be it known that I, ANSON GARDNER BETTS, a citizen of the United States, residing at Troy, in the county of Rensselaer and State of New York, have invented certain new and useful Improvements in Electrolytically Refining Silver, of which the following is a specification accompanied by a drawing.

Reference may be had to the accompanying drawing, and the reference characters marked thereon, which forms a part of this specification.

Similar characters refer to similar parts in the drawing.

The single figure of the drawing is a view in vertical cross-section of an electrolytic cell for carrying out my invention.

This invention relates to the use of solutions of silver salts of strong non-oxidizing, preferably monobasic, acids, as electrolytes for electrolytically refining silver alloys.

Certain objects of my invention are to produce a silver deposit on the cathodes of such solidity that the electrolytic refining operation and apparatus are respectively facilitated and improved, and to effect the solution of antimony, bismuth, and such usually undesirable elements of the anodes with the silver.

Other objects may be noted in the following description.

Such objects are achieved by using in the electrolytes strong non-oxidizing acids, and, further, by the addition of small amounts of certain substances, as gelatin and gum-arabic. These substances should most suitably be present between the proportions of one part to twelve thousand solution and one part to fifteen thousand. The presence of oxidizing compounds—nitric acid, for example—is found to prevent the action of the gelatin or gum in preventing the growth of the deposits on the cathodes toward the anodes. An especially suitable solution contains four per cent. silver, as silver methyl sulfate, and four per cent. of methyl sulfuric acid. When silver has been reduced to one and one-half per cent., from the presence of lead, copper, or bismuth in the anodes, the solution should be removed and replaced by fresh solution. Other suitable acids are fluoroboric, alkyl sulfonic, and sulfuric acids, and aromatic sulfonic acids.

Dithionic acid gives good results, as it is a strong acid, somewhat stronger than sulfuric acid; but the results with any dibasic acid are distinctly inferior to those obtained with mon-

obasic acids of the strongest order, such as I have mentioned.

The electrolysis may be very well carried on with a current density of ten amperes per square foot cathode surface for as long a time as the high value of silver under treatment makes economical—say forty-eight hours—without the least danger of short-circuiting from the growth of “trees.” The deposit is not perfectly solid and can be easily scraped off the cathode sheets, which I have found to be an advantage rather than otherwise, for the cathode sheets may be used over and over again. No silver falls from the cathodes into the tanks or when removing them, unless it is knocked off with some instrument.

No necessity exists for wrapping silver anodes in cloth, as in hitherto used electrolytic parting processes, for whether the anode slime, mostly of gold, drops from the anodes or remains sticking to them it cannot become mixed with the cathode silver.

A particular advantage in using strong non-oxidizing monobasic acids is that they dissolve large quantities of their bismuth salts, and a considerable excess of free acid does not cause any action on the electrodes beyond the electrolytic action. The bismuth accumulating in the solution I can precipitate with hydrofluoric acid, as bismuth fluorid; or after precipitating silver—for instance, with metallic bismuth—by precipitation with metallic lead. If the latter method is adopted, the resulting lead solution can be treated with finely-divided silver sulfate, precipitating lead sulfate and regenerating silver solution to be used over again.

Having reference to the accompanying drawing, 1 is a tank containing the electrolyte 2.

In the electrolyte are suspended anodes 3 of silver containing impurities and cathodes 4, on which is the pure electrodeposited silver 5.

What I claim as new, and desire to secure by Letters Patent, is—

1. The process of electrolytically refining silver which consists in subjecting the silver alloy as anode to an electric current in an electrolyte containing a free, non-oxidizing, strong acid forming a readily-soluble silver salt, and the silver salt of said acid, and electrolytically depositing the silver on a suitable cathode.

2. The process of electrolytically refining silver which consists in subjecting the silver

alloy as anode to an electric current in an electrolyte containing a free, non-oxidizing, monobasic strong acid forming a soluble silver salt, and the silver salt of said acid, and electrolytically depositing the silver on a suitable cathode.

3. The process of electrolytically refining silver which consists in subjecting the silver alloy as anode to an electric current in an electrolyte containing a free, non-oxidizing, monobasic strong acid forming a soluble silver salt, the silver salt of said acid, and an agent to hinder the growth toward the anode of the cathode deposit of silver, and electrolytically depositing the silver on a suitable cathode.

4. The process of electrolytically refining silver containing bismuth which consists in subjecting the silver alloy as anode to an electric current in an electrolyte containing a free, non-oxidizing, monobasic strong acid, the silver salt of said acid, and an agent to hinder the growth toward the anode of the cathode deposit of silver, and electrolytically depositing the silver on a suitable cathode; and recovering from the electrolyte the bismuth dissolved from the anode.

5. The process of electrolytically refining silver containing bismuth which consists in subjecting the silver alloy as anode to an

electric current in an electrolyte containing a free, non-oxidizing, monobasic strong acid, the silver salt of said acid, and an agent to hinder the growth toward the anode of the cathode deposit of silver, and electrolytically depositing the silver on a suitable cathode; and recovering by precipitation with metallic lead, the bismuth dissolved from the anode.

6. The process of electrolytically refining silver containing bismuth which consists in subjecting the silver alloy as anode to an electric current in an electrolyte containing a free, non-oxidizing, monobasic strong acid, the silver salt of said acid, and an agent to hinder the growth toward the anode of the cathode deposit of silver, and electrolytically depositing the silver on a suitable cathode; recovering bismuth dissolved from the anode from the electrolyte by precipitation with metallic lead, precipitating lead from the electrolyte, dissolving silver in the electrolyte, and using the thus regenerated electrolyte in electrolytically refining silver.

In testimony whereof I have signed my name to this specification in the presence of two subscribing witnesses.

ANSON GARDNER BETTS.

Witnesses:

LIVERMAN P. SHOTTEN,  
EDWARD F. KERN.